

July 7, 1959

E. WALASCHEWSKI ET AL

2,893,862

PROCESS FOR THE PRODUCTION OF ALKALINE-EARTH METALS

Filed Sept. 19, 1956

2 Sheets-Sheet 1

FIG.1



INVENTORS

Engelbert Walaschewski, Dieter Goerrig  
BY *Bürgen, Linklage & Sprung*  
ATTORNEYS

July 7, 1959

E. WALASCHEWSKI ET AL

2,893,862

PROCESS FOR THE PRODUCTION OF ALKALINE-EARTH METALS

Filed Sept. 19, 1956

2 Sheets-Sheet 2



FIG. 2



FIG. 3



FIG. 4



FIG. 5



FIG. 7



FIG. 6



FIG. 8

INVENTOR.

ENGELBERT WALASCHEWSKI, DIETER GOERRIG

BY

Bürgers, Dinklage & Sprung  
ATTORNEYS

# United States Patent Office

2,893,862

Patented July 7, 1959

1

2,893,862

## PROCESS FOR THE PRODUCTION OF ALKALINE-EARTH METALS

Engelbert Walaschewski, Köln-Bayenthal, and Dieter Goerrig, Lohmar, Germany, assignors to Farbenfabriken Bayer Aktiengesellschaft, Leverkusen, Germany, a corporation of Germany

Application September 19, 1956, Serial No. 610,812

Claims priority, application Germany September 26, 1955

8 Claims. (Cl. 75—67)

This invention relates to a process for the production of alkaline-earth metals.

It is known, in the production of alkaline-earth metals, that it is possible to heat alkaline-earth hydrides, whereby hydrogen is split off and the alkaline-earth metal is left in a more or less pure form, depending on the amount of impurities in the hydride. When the metal thus obtained is distilled, the major part of the impurities are left behind, but it is not possible to obtain a very pure metal in this way, since the distillate always contains nitrogen.

The present invention is concerned with a process for the production of pure alkaline-earth metals by heating alkaline-earth hydrides and distilling the alkaline-earth metal which is obtained, the said process consisting in preventing nitrogen from acting on the distilling metal. It has surprisingly been found that the nitrogen present in the hydride does not pass over with the distilling metal if the starting material subjected to the heating contains such a high content of aluminum that the nitrogen is fixed in the form of aluminium nitride.

In addition to the splitting of alkaline-earth hydrides into hydrogen and alkaline-earth metal, a number of other reactions take place during the thermal decomposition; thus, carbon, which may be present in elementary form or as carbonate, changes into alkaline-earth carbide, sulphur into sulphide and silicon compounds into silicides. These reactions all lead to compounds which are considerably less volatile than the alkaline-earth metals. The nitrogen compounds of the alkaline-earth metals, however, decompose under the temperature and pressure conditions of the vaporisation of the metal and reform under the conditions under which the metal is condensed. For the production of pure alkaline-earth metals, it is consequently of decisive importance that the nitrogen in the material to be distilled can be fixed as aluminium nitride, since aluminium nitride has such a high decomposition temperature that the distillation of the alkaline-earth metals can take place without nitrogen being simultaneously split off.

The amount of aluminium or aluminium compounds, such as alumina, or aluminium alloys, such as calcium-aluminium, which must be admixed with the initial material, which is to be distilled, depends of course on the amount of nitrogen contained in the initial hydride. If the initial hydride contains aluminium, the amount of aluminium to be added is reduced accordingly; in certain circumstances, the separate addition of aluminium is unnecessary, if the crude hydride contains a sufficient amount of aluminium to ensure that the nitrogen present is fixed as nitride, for example 1.52% Al and 0.28% N.

On heating the alkaline-earth hydrides to 1000–1150° C. at normal pressure, about 50% of the hydrogen present is split off, while the major part of the residual hydrogen is split off with further heating at 1150–1350° C. with formation of more or less highly impure liquid alkaline-earth metals, which start to vaporise at temperatures above 1400° C. and yield a pure metal condensate when the distillation is completed at 1600° C. The proc-

2

ess is advantageously carried out at reduced pressure, so that the splitting and distillation is carried out at temperatures below 1000° C. and pressures of a few hundred mm. Hg to less than 10<sup>-2</sup> mm. Hg.

5 The pure alkaline-earth metal thus produced and distilled in the presence of aluminium still always contains nitrogen, even if in very small quantities. The occurrence of these amounts of nitrogen is avoided according to the invention if the metal vapour is passed through highly 10 efficient dust separators, for it was established that nitrogenous fractions in powder form are extracted by the distillation from the solid phase and are included in the metal in the condensation. There are employed as dust separators combinations of filters such as are used in 15 moderate coarse vacuum and high vacuum work.

Very small amounts of nitrogen are still present in the alkaline-earth metal which is condensed after extremely 20 careful filtration of the metal vapour. According to the invention, an alkaline-earth metal is obtained which is practically completely free from nitrogen if the decomposition of the hydride and the distillation of the metal is carried out in apparatus of which the outer walls are 25 cold; it has in fact been found that the said small amounts of nitrogen result from diffusion of nitrogen through hot apparatus walls. According to the invention, for example 30 apparatus having double walls are used, insulating material being provided between the said walls in order that the rise in temperature of the outside walls is kept within narrow limits or is completely prevented.

The process according to the present invention is excellently suitable for the production of alkaline-earth 35 metals from the technical hydrides which can be obtained according to conventional methods.

One embodiment of an apparatus which can be used 40 for the preparation of ultra-pure alkaline-earth metals according to the invention is illustrated in the accompanying drawings.

Figure 1 is a longitudinal sectional view of the 45 apparatus.

A reaction vessel 1 is heat-insulated by means of an insulation 2 inside which is arranged a chrome-nickel vessel 3 adapted to be heated to the reaction temperature by the electrical heating system 4. Arranged at the base of the reaction vessel is a supply pipe 5 for argon or another inert gas, while a connection 6 for a vacuum pump 50 is provided at the top of the reaction vessel 1. Projecting from above into the reaction vessel 1 is a cooling arrangement 7 with supply and discharge devices 8 and 9 for a coolant, such as cooling water. The distilled metal 10 is precipitated at this cooling arrangement. The starting material 11 is located at the bottom of the chrome-nickel vessel 3. The metal distilled out of the said material 11 passes in gaseous form through the dust filter 12. A circulation pump 13 is provided between the vacuum connection 6 and the argon supply pipe 5.

55 Figure 2 is a plan view and Figures 3 and 4 are cross-sections of filter arrangements for the dust precipitation, the said filters consisting essentially of inclined metal plates 14 and a metal screen 15, it being possible for the 60 said screen 15 to be arranged below the inclined metal plates 14, as shown in Figure 3, or above said plates, as shown in Figure 4.

Figure 5 is a plan view and Figure 6 is a cross-section of another constructional form of a dust separator, this 65 consisting essentially of perforated plates 16 with perforations offset from one another and a metal screen 15.

Another constructional form of a dust separator is shown in Figures 7 and 8, Figure 7 being a plan view and Figure 8 a cross-section. It consists essentially of two or more concentric annular discs arranged in spaced 70 superposed relation, the diameters thereof decreasing in the upward direction; the discs 17 are covered by a plate

18 which is also arranged in spaced relation. A metal screen 15 is disposed underneath the said arrangement.

The invention is further illustrated by the following example without being restricted thereto.

*Example 1*

12.5 kg. of technical calcium hydride of the composition (in percent by weight)

|              |       |
|--------------|-------|
| Ca           | 83.19 |
| H            | 3.62  |
| C            | 1.94  |
| O            | 5.71  |
| N            | 0.88  |
| S            | 0.93  |
| P            | 0.01  |
| Si           | 1.24  |
| Ac           | 1.68  |
| Fe and other | 0.80  |

with an effective calcium hydride content of 72-73% is placed in the apparatus described above after having had added thereto 0.125 kg. of an aluminium-calcium alloy containing 50% of aluminium, and with the vacuum pump cooperating with a suction capacity of 50 cu. metres per hour, the mixture is heated by the electric heating system with a heating capacity of 8 kw. After 3 hours, a temperature of 900° C. and a pressure of 0.1 mm. Hg are reached. After switching on two mercury diffusion pumps, heating is continued for another hour with the full heating capacity and a pressure lower than 10<sup>-2</sup> mm. Hg until the temperature suddenly starts to rise to just 1000° C. The furnace is then cooled by pumping argon at a pressure of 6 atm. gauge by means of a circulation compressor through the furnace. 8.1 kg. of calcium metal with a purity of 99.98% are obtained at the cooling arrangement.

Total analysis yields:

|                        | Percent             |
|------------------------|---------------------|
| Ca                     | About 99.98         |
| Sr                     | About 0.005         |
| Ba                     | Below 0.001         |
| Mg                     | About 0.005         |
| Na+other alkali metals | About 0.001         |
| Si                     | Below 0.001         |
| Al                     | Below 0.001         |
| V+Mn                   | About 0.005         |
| Fe and other metals    | Below 0.001         |
| N                      | About 0.0002-0.0004 |
| O                      | Below 0.001         |
| C                      | Below 0.001         |
| H                      | About 0.005         |

Analogous results are obtained when barium hydride with 52% BaH<sub>2</sub> and a strontium hydride with 55% of SrH<sub>2</sub> are processed in the same way.

We claim:

1. In the process for the production of an alkaline-earth metal having an atomic number between 20 and 56 by thermally splitting an alkaline-earth metal hydride into hydrogen and the respective alkaline-earth metal and distilling the alkaline-earth metal the step which comprises

fixing the nitrogen present in the starting material in the form of aluminum nitride by performing the process in the presence of such an amount of aluminum which is at least chemically equivalent to the nitrogen amount present in the starting material.

2. In the process for the production of an alkaline-earth metal having an atomic number between 20 and 56 by thermally splitting an alkaline-earth metal hydride into hydrogen and the respective alkaline-earth metal and distilling the alkaline-earth metal the step which comprises fixing the nitrogen present in the starting material in the form of aluminum nitride by performing the process in the presence of such an amount of aluminum which is at least chemically equivalent to the nitrogen amount present in the starting material and filtering the earth-alkaline metal vapour so as to prevent the entraining of nitrogen containing dust into the distillate.

3. In the process for the production of an alkaline earth metal having an atomic number between 20 and 56 by thermally splitting an alkaline earth metal hydride containing such an alkaline earth metal into hydrogen and the respective alkaline earth metal, and distilling the alkaline earth metal the step which comprises fixing the nitrogen present in the starting material in the form of aluminum nitride by performing the process in the presence of such an amount of an aluminum material selected from the group consisting of aluminum, an aluminum compound and an aluminum alloy, which is at least chemically equivalent to the nitrogen amount present in the starting material.

4. Process according to claim 3 in which said alkaline earth metal hydride is calcium hydride.

5. Process according to claim 3 in which said alkaline earth metal hydride is barium hydride.

6. Process according to claim 3 in which said alkaline earth metal hydride is strontium hydride.

7. Process according to claim 3 which includes filtering the earth alkaline metal vapor so as to prevent the entraining of nitrogen containing dust into the distillate.

8. In the process for the production of an alkaline earth metal having an atomic number between 20 and 56 by thermally splitting an alkaline earth metal hydride containing such an alkaline earth metal into hydrogen and the respective alkaline earth metal and distilling the alkaline earth metal, the step which comprises fixing the nitrogen present in the starting material in the form of aluminum nitride by performing the process in the presence of such an amount of an aluminum material selected from the group consisting of aluminum, an aluminum compound and an aluminum alloy, which is at least chemically equivalent to the nitrogen amount present in the starting material and keeping the outer wall of the reaction space at a low temperature so as to prevent nitrogen from diffusing into the reaction space.

**References Cited in the file of this patent**

**UNITED STATES PATENTS**

|           |          |               |
|-----------|----------|---------------|
| 2,276,239 | Nelson   | Mar. 10, 1942 |
| 2,402,193 | Willmore | June 18, 1946 |
| 2,448,000 | Kemmer   | Aug. 24, 1948 |